

Patented Dec. 26, 1939

2,185,125

BEST AVAILABLE COPY

# UNITED STATES PATENT OFFICE

2,185,125

## METHOD OF COATING PRINTED SURFACES AND ARTICLE FORMED THEREBY

Roy E. Coleman, Meriden, Conn., assignor to The  
Zein Corporation of America, a corporation of  
Delaware

No Drawing. Application November 22, 1937,  
Serial No. 175,888

10 Claims. (Cl. 91—67.9)

This invention relates to methods of coating printed surfaces and more particularly to methods of coating printed labels with protective varnishes made from zein or other prolamins and to the article produced thereby. The invention set forth herein is related to the invention described in my copending application Serial No. 158,215, filed August 9, 1937.

In the following description of the method embodying my invention I will refer to the preparation of substantially non-aqueous varnish compositions made from zein derived from corn, but it is to be understood that my invention is also applicable to the preparation of varnish compositions made from the other prolamins such as, for example, gliadin from wheat, hordein from barley, kafirin from kafir and the prolamins from other cereal grains. The above-mentioned prolamins are at present derived by extraction with an aqueous alcohol solution in which the added water varies generally from about 15 to about 40% of the solvent mixture. The material utilized in preparing the varnishes used in accordance with my invention is the dried extract which may be completely dried or the commercial product which contains a small percentage of moisture.

In carrying out my invention, a printed surface such as, for example, a label, carton, advertising card, playing card, magazine cover and the like, printed with, for example, an oleaginous base type of ink, is covered with a thin, flexible, transparent film of a zein varnish, suitably by machine coating, dipping, spraying or over-printing process or by other suitable coating process. The varnish film formed of such varnish dries in a relatively short time, in the order of about 2 to 60 minutes at room temperature, owing to the fact that zein solutions give up their solvent with extraordinary readiness; and they form a hard, transparent film having a high gloss which appears to accentuate and intensify the underlying printed matter. This drying time may be materially hastened by the application of heat and is, of course, influenced by the characteristics of the solvents utilized in effecting solution of the zein, by modifying agents, by the thickness of the film, etc.

In general, the usually dry zein varnish films are compatible with glue or similar water-soluble adhesive materials. Hence the dried zein varnish films present a surface that may be coated with glue which, on hardening, is capable of forming a strong, adherent layer on the varnish films. This characteristic of the films formed in

accordance with the method embodying my invention renders the method especially suitable for label printing, since the necessity for the provision of an unvarnished area to which glue may be applied, as in the prior art, is eliminated. In accordance with the prior art practice, a localized unprinted and unvarnished area on a label is necessary so that glue may be applied and adhere thereto for the purpose of securing the label around a can or the like, since glue is not compatible with and does not adhere to the usual oleaginous materials comprising the ink base or the usual varnish coatings. In practice, the labels are first printed with the desired design and a localized, unprinted area is provided to which the glue may be applied. After drying, the printed labels are coated with a protective varnish over all but the unprinted localized area by means of a printing machine, as an overprint varnish. This practice is objectionable from the standpoint of the time required to overprint in registry with the printed area to be protected by the varnish, the difficulty of preventing off-setting, and the drying time and these requirements render the process costly.

In accordance with my present invention, these objections are overcome by the provision of a zein film as the protective coating, which may be applied as an all-over coating by any of the conventional coating processes. The zein protective coating readily adheres to any printed surface, even when an oleaginous base type of ink has been used for the printing, and dries rapidly. The glue may then be applied to the desired localized area of the zein film for securing the label to the desired object and on drying, the glue forms a perfect bond with the zein surface. Accordingly, by operating in accordance with my invention a substantial saving of time is effected and the objections to the overprinting and varnishing as in the prior art are obviated.

The printed labels, magazine covers and the like, when coated with the zein varnish in accordance with my method, appear to resist curling or crinkling when in contact with water or aqueous mediums. They are substantially as flexible as the untreated labels, magazine covers and the like and, in some instances, more so; and have a marked resistance to oleaginous materials.

The varnish compositions used in accordance with the present invention are substantially non-aqueous solutions of zein containing preferably from 0 to 5% of added water. While the inclu-

- sion of larger percentages of water is not precluded, I have found that the field of applicability of the varnish compositions decreases as the water content thereof increases. These compositions are stable, in so far as separation is concerned, at temperatures of 70° F. and below and in many instances at temperatures of 40° F. and below and do not have a marked tendency to thicken and gel on standing.
- 10 The following examples are illustrative of the varnish compositions which may be used in accordance with my invention to produce a zein varnish protected printed surface, and it is to be understood that other varnish compositions 15 in other proportions may be used in accordance with my invention all as hereinbefore set forth. In the examples, the term "parts" indicates parts by weight.

*Example 1*

- 20 10 parts of zein are mixed with 30 parts of propylene glycol. On stirring the mixture at room temperature the zein mixes readily with the propylene glycol but does not dissolve. On heating 25 to about 160° to 190° F. a perfectly clear, transparent, bright, stable zein varnish is obtained in about 8 to 15 minutes. This varnish is coated onto a printed surface in a conventional coating machine and the coating dries in about 30 to 60 minutes to form a transparent, strongly adherent film which is both hard and flexible and has a very high gloss. The zein varnish renders the printed surface moisture and oil 35 resistant.

*Example 2*

- 40 10 parts of zein are mixed with 40 parts of diacetone alcohol (acetone free) and heated in the order of about 165° to 190° F. to form a colloidal, slightly cloudy zein varnish composition. 45 This varnish, on cooling and standing becomes quite viscous but turns transparent and remains stable.

This varnish is now applied onto a printed label either on a coating machine, or by overprinting and in about 15 to 20 minutes the coating dries to a transparent, flexible, strongly adherent film having a high gloss. The film renders the label substantially moisture and oil 50 resistant and accentuates the printed matter appearing thereon.

*Example 3*

- 55 10 parts of zein are mixed with 40 parts of a solvent mixture containing 10% of ethylene glycol monomethyl ether and 90% of 95% alcohol. On stirring and with the application of heat in the order of about 90° to 120° F., a stable zein varnish is obtained in about 8 to 12 minutes.

This composition is now thinned, as by the addition of the solvent mixture, until the varnish 60 has a viscosity suitable for use in a spray gun. The thinned varnish is then sprayed onto a label or printed magazine cover and in about 5 minutes the coating dries to a hard, flexible, transparent film having a very high gloss. The zein varnish film renders the label or magazine cover 65 moisture and oil resistant, and both accentuates and intensifies the printed matter on the coated surface.

*Example 4*

- 70 10 parts of zein are mixed with 40 parts of diacetone alcohol (acetone free) and 6 parts of lauric acid. In practice, the zein is mixed with the diacetone alcohol and heated to about 165 to 75 190° F., for about 8 to 12 minutes to effect solu-

tion. The solution is then cooled to about 130 to 140° F., and the lauric acid is then added to form a stable zein varnish.

The varnish is applied to a printed label as by over-printing and in about 10 to 15 minutes a clear, transparent, hard and glossy film is formed which imparts both moisture and oil resistance to the label.

The films produced on the printed surfaces as above described have no after-tack, will not soften on heating and are, for all practical purposes, scratch-proof. Zein film to film or film to paper bonds may be effected with any of the conventional water-soluble glues or adhesives.

In carrying out the process according to my invention a decided advantage inures to the operator since the zein varnishes used in accordance with my invention have the unusual property of being able to dissolve in themselves even after having remained and dried on the coating rolls or other coating machinery. By virtue of this fact the coating machinery parts need not be cleaned of coating materials immediately after the end of a run or after a break-down as is now required in the prior art processes.

The characteristics of the varnish compositions used in accordance with my invention and hence of the ultimate protective films can be altered at will and as desired by the inclusion in the varnish composition of diluents, modifiers, plasticizers and the like as set forth in my above-identified copending application. The characteristics, such as spread and flow, of these varnishes may also be modified by the addition of a fatty acid such as, for example, oleic, linseed, hemp seed, lauric and like fatty acids and by the inclusion of cetyl, lauryl, myristyl and like fatty alcohols having 8 or more carbon atoms in the chain. If desired, compatible natural and synthetic resins such as for example, rosin, sandarac, 40 copal, phenol-aldehyde, urea-aldehyde, glycerine-phthalic anhydrid, vinyl and like resins, or compatible cellulose derivatives such as, for example, high and low viscosity nitrocellulose, cellulose acetate, ethyl cellulose and like cellulose derivatives may be incorporated with these zein varnishes in varying proportions to meet the desired needs.

In the claims when I use the expression "substantially non-aqueous" I refer to varnish compositions made from zein or the other prolamins wherein the added water is preferably 5% or less. When I use the expression "stable" I mean varnish compositions which do not separate on standing or even when cooled to temperatures 55 of 50 to 70° F. and somewhat below. The stable substantially non-aqueous varnishes are capable of drying to a clear, transparent flexible, and hard film.

I claim:

1. The method of protecting a printed surface which comprises coating the printed surface with a zein varnish capable of drying to a hard, transparent film, said varnish containing not in excess of 5% of water.

2. The method of applying a protective coating layer to a printed label which comprises coating the printed surface of the label with a zein varnish capable of drying to a hard, flexible, transparent film, said varnish containing not in excess of 5% of water.

3. The method of applying a protective coating layer to a printed label which comprises coating the printed surface of the label with a varnish comprising zein and propylene glycol capable of

drying to a hard, glossy, flexible, transparent film, said varnish containing not in excess of 5% of water.

4. The method of applying a protective coating layer to a printed label which comprises coating the printed surface of the label with a varnish comprising zein and diacetone alcohol capable of drying to a hard, glossy, flexible, transparent film, said varnish containing not in excess of 5% of water.

5. The method of applying a protective coating layer to a printed label which comprises coating the printed surface of the label with a varnish comprising zein, diacetone alcohol and lauric acid capable of drying to a hard, glossy, flexible, transparent film, said varnish containing not in excess of 5% of water.

6. The method of applying a protective coating layer to a printed label which comprises coating the printed surface of the label with a varnish comprising zein, ethylene glycol monomethyl ether and 95% alcohol capable of drying to a hard, glossy, flexible transparent film, said varnish containing not in excess of 5% of water.

25 7. A printed label carrying a hard, flexible, glossy, transparent zein coating layer over the

printed matter, said coating layer being adapted to receive a coating of glue capable of drying to a hard, adherent layer on said zein coating layer, said layer being deposited from a liquid zein coating composition containing not in excess of 5% of water.

8. A printed label carrying a hard, flexible, glossy, transparent prolamin coating layer over the printed matter, said layer being deposited from a liquid prolamin coating composition containing not in excess of 5% of water.

9. A label printed with an oleaginous base type of ink carrying a hard, flexible, glossy, transparent zein coating layer over the printed matter and a coating of glue along a localized area of the zein film, said layer being deposited from a liquid zein coating composition containing not in excess of 5% of water.

10. The method of printing and coating a label comprising, printing a label with an oleaginous base type of ink, coating the printed surface with a liquid zein composition containing not in excess of 5% of water and which is capable of adhering to the printed surface and coating a localized area of the zein surface with glue.

25 ROY E. COLEMAN.